

Jan. 14, 1958

F. A. HAMM

2,819,963

LIGHT SENSITIVE COMPOSITION FOR PHOTOMAGNETIC PRINTING PROCESS

Filed Jan. 7, 1955

**Fig.1**



EXPOSE

**Fig.2**



DEVELOPMENT & ETCH

**Fig.3**



**Franklin A. Hamm**

INVENTOR.

BY *Daniel J. Maguire*

*Lawrence H. Willis*

ATTORNEYS

1

2,819,963

## LIGHT SENSITIVE COMPOSITION FOR PHOTO-MAGNETIC PRINTING PROCESS

Franklin A. Hamm, Rochester, N. Y., assignor to Eastman Kodak Company, Rochester, N. Y., a corporation of New Jersey

Application January 7, 1955, Serial No. 480,489

7 Claims. (Cl. 96—94)

This invention relates to the preparation of photographic resist materials and to methods of forming images therefrom.

The use of bichromated glue for preparing resists in the photoengraving industry is well known, and such materials have been used for many years. It is also well known that a pigment can be incorporated in the sensitized glue and a pigmented image thereby obtained. In the preparation of an image in this way, the coating of pigmented colloid must necessarily be quite thin so that exposure to light will harden the colloid throughout its entire thickness and the hardened portions will then adhere to the support upon washing with water. The unexposed portions will dissolve away and this process will yield a positive from a negative.

The material of my invention can be applied easily to most supports and can be processed in a simple manner. Its speed range is ideal for practical purposes, and it can be handled and coated in safe light. Other advantages of my process and material will be evident from the following description of my invention.

Accordingly, one object of my invention is to provide superior light-sensitive materials for making photographic resists which can be used as printing plates. Another object is to provide photographic resist materials which can be used for long periods of time without degradation of the printing surface. Still another object of my invention is to provide photographic resists which give a number of copies from the same printing surface, each of the copies being characterized by superior resolution and sharpness. Other objects will become apparent from a consideration of the following description and examples.

In practicing my invention, a ferromagnetic iron oxide, such as gamma ferric oxide ( $Fe_2O_3$ ) or ferroso-ferric oxide ( $Fe_3O_4$ ), is uniformly dispersed in a photographic gelatino-silver-halide emulsion and the mixture is coated uniformly on a surface. The photographic emulsion is then exposed in the usual manner and processed to a relief image. The relief image is then magnetized or sensed, developed with finely divided iron (ferromagnetic) and copies obtained by contact transfer printing, for example. Although a relief or resist image is formed in the silver-halide emulsion layer, it is the magnetic property of the iron oxides which is the important aspect in the production of copies from the master. The quality of the master is not impaired by light, heat, moisture, or pressure. The magnetism is not inadvertently erased.

In the accompanying drawing, the various figures show in enlarged cross-sectional view the structure of a representative sensitive element of my invention at various stages in the process of producing printing plates having select areas covered by the resist images.

The quantity of ferromagnetic iron oxide dispersed in the photographic silver-halide emulsion layer can be varied, depending upon the type of copy which is to be produced. The optimum quantity for a given purpose can be ascertained by making a series of test strips containing various quantities of ferromagnetic oxide. In gen-

2

eral, the speed of the photographic gelatino-silver-halide emulsion containing the ferromagnetic iron oxide is about one-third of that of a similar photographic emulsion containing no ferromagnetic iron oxide.

5 The relief image which is employed for printing according to my process can be obtained by either tanning development or regular development, followed by treatment with an etch-bleach bath. These alternative methods of processing are discussed in detail below. Other 10 methods of obtaining a relief image can also be employed, depending upon the use to which the relief image is to be put.

The relief image thus formed is magnetized or sensed using a recording head so that the relief image is now

15 also a magnetic image. This magnetization can be accomplished in known manner, at various A. C. frequencies and speeds of motion of the magnetic matrix. However, the condition of 250 cycles/second, 8 volts, 90 milliamperes, and a speed of about 2-3 inches per second 20 has proved to be very satisfactory. Contact recording (sensing) is desirable. Other methods of magnetizing the relief record can be employed equally well. Such methods of magnetization are matters of common knowledge.

The magnetic latent image thus obtained is then "developed" to a magnetic visible image using finely divided iron (ferromagnetic). A suspension of this free iron (sometimes referred to as a magnetic ink) in carbon tetrachloride or other vehicle can be flooded over the relief image, or the master image can be immersed in the 30 suspension. In both cases, the magnetic lines of force in the magnetized relief image attract the soft iron (ferromagnetic) particles and hold them firmly in contact with the relief image. Regions in the master which are void of the ferromagnetic iron oxide matrix are free of developing iron. Also, the amount of iron attracted to regions in the relief image will be somewhat dependent on the thickness of the image at any given region.

Copies can best be made by contact transfer. One 35 method comprises using a moist, pressure-sensitive adhesive transfer material, such as dye transfer paper. The dye transfer paper is slightly moistened on the gelatin side and this side is placed in contact with the developed master. Gentle pressure results in transfer of the iron from the surface of the master matrix to the gelatin surface of the dye transfer paper. There is thus obtained an image 45 on the transfer paper which consists of free iron embedded in gelatin. The record thus obtained can be preserved by spraying with a solution of an organic solvent containing dissolved resin, such as polymethyl methacrylate, poly- 50 methyl acrylate, etc.

Alternatively, transfer of the image from the resist material to a desired surface can be accomplished by placing the master image in contact with dry dye transfer paper with the gelatin coating thereof in contact with 55 the developed master. When dry heat is applied to the rear surface of the dye transfer paper, transfer of the iron from the master surface occurs. A heat-sealing iron can also be used.

The following example will serve to illustrate further 60 the manner of practicing my invention.

### EXAMPLE

Six parts by weight of gamma ferric oxide were mixed with about 4 parts by weight of a photographic gelatino-silver-halide emulsion and the dispersion coated on a photographic support, such as cellulose acetate.

#### (a) Tanning development

A photographic element obtained as described above 70 was exposed to a line image through the base. The exposed emulsion layer was then developed for two minutes in a tanning developer of the type described in John

U. S. Patent 1,482,613, issued February 5, 1924 (see page 2, column 2, lines 25-35). Following development, the emulsion was subjected to a 3-minute wash in running water at 140° F.

(b) *Regular development*

A second photographic element was made as described above and exposed to a line image in the conventional way through the photographic emulsion layer instead of the base. The exposed emulsion layer was then developed for 4 minutes in Kodak Developer D-19. The developed emulsion was then fixed and washed in the usual manner.

The emulsion layer was then subjected for 45 seconds to an etch-bleach bath of the following composition:

Part A:

|                        |       |     |
|------------------------|-------|-----|
| Cupric nitrate         | grams | 200 |
| Potassium bromide      | do    | 10  |
| Glacial acetic acid    | cc    | 160 |
| Water to make 1 liter. |       |     |

Part B: 3% hydrogen peroxide solution.

Equal parts by volume of A and B above were mixed immediately before use.

After the silver emulsion was completely bleached by the above solution, the outer surface of the element was gently washed with water and the resulting relief image allowed to dry.

(c) *Making copies*

The relief image which had been obtained in part a (or part b) above was sensed magnetically by passing the relief image past a magnetic recording head which had been positioned in the chuck of a milling machine. The table speed was 2.5 inches per second and the length of the air gap in the recording head was 1.96 mils. The gap width was about 0.75 mil. The displacement normal to the motion of the milling machine was indexed to 150 mils so that an overlap of 46 mils occurred during each track length. In order to avoid white separation lines in the printed copies, it was found that the length of the magnetic recording head should be made approximately equal to the width of the area to be magnetized. Magnetic erasure is thus avoided.

The resist image which had thus been magnetically sensed was then treated with powdered iron (ferromagnetic) as described above. Carbonyl Iron, Type G, sold by the General Aniline and Film Corporation was found to be useful as the "developing" iron. It was found to be about 98% pure and to have a weight-average diameter of about 8 microns. It was spherical in form. The developed image was then placed in contact with dye transfer paper and an image of excellent resolution obtained. Since exposure is generally made through the base or support when a tanning development is employed, the image obtained is a negative of the original image and its left-right directions are reversed with respect to the original. When the regular development and etch-bleach treatment are employed, the exposure is from the emulsion side, and the copy is a positive of the original and has correct orientation.

The process of my invention is most advantageously suited for line copies. If desired, copies can be made of an original by exposure in a camera in the ordinary manner or exposure can be made through a negative or positive in the usual manner. The quality of the copies can be improved somewhat in those cases where transfer is affected to a support having thereon a gelatin layer by applying slight pressure to the rear side of the support having thereon the gelatin layer. While the above example employed a photographic gelatino-silver-halide emulsion wherein the halide was bromide, other silver

halides can be employed to advantage, such as the ordinarily employed gelatino-silver-chloride, gelatino-silver-bromide, gelatino-silver-chlorobromide, gelatino-silver-bromide, etc. emulsions.

5 Kodak Developer D-19 has the following composition:

|                                      |       |      |
|--------------------------------------|-------|------|
| Water, about 125° F. (50° C.)        | cc    | 500  |
| Kodak Elon developing agent          | grams | 2.0  |
| Kodak sodium sulfite, desiccated     | do    | 90.0 |
| Kodak hydroquinone                   | do    | 8.0  |
| Kodak sodium carbonate, monohydrated | do    | 52.5 |
| Kodak potassium bromide              | do    | 5.0  |
| Cold water to make 1.0 liter.        |       |      |

My invention can be further illustrated by reference to 15 the accompanying drawing. Figure 1 shows a support 10

of any suitable material, such as cellulose acetate, polyvinyl acetal, etc., coated with a layer 11 containing a photographic gelatino-silver-halide emulsion having dispersed therethrough a ferromagnetic iron oxide, such as gamma 20 ferric oxide. In Figure 2 the light-sensitive material shown in Figure 1 has been exposed to light under an image having transparent portions 13 and opaque portions 12. After development of the exposed element 25 shown in Figure 2 and treatment with an etch-bleach bath as shown above, there is obtained the resist image shown in Figure 3. The image consists of raised portions 14 containing gamma ferric oxide or other ferromagnetic material. This resist image can then be magnetized as described above and the magnetized surface 30 treated with iron powder to produce a visible record of the subject. This visible record can then be transferred to another surface, such as dye transfer paper as described in detail above.

What I claim as my invention and desire secured by 35 Letters Patent of the United States is:

1. A photomechanical resist composition comprising a photographic gelatino-silver-halide emulsion and a ferromagnetic iron oxide.
2. A photomechanical resist composition comprising a photographic gelatino-silver-halide emulsion and gamma ferric oxide.
3. A photomechanical resist composition comprising a photographic gelatino-silver-bromide emulsion and gamma ferric oxide.
4. A photographic element comprising a support having thereon a layer comprising a photographic gelatino-silver-halide emulsion and a ferromagnetic iron oxide.
5. A photographic element comprising a support having thereon a layer comprising a photographic silver-halide emulsion and gamma ferric oxide.
6. A photographic element comprising a support having thereon a layer comprising a photographic gelatino-silver-bromide emulsion and a ferromagnetic iron oxide.
7. A photographic element comprising a support having thereon a layer comprising a photographic gelatino-silver-bromide emulsion and gamma ferric oxide.

References Cited in the file of this patent

| UNITED STATES PATENTS |         |               |
|-----------------------|---------|---------------|
| 494,526               | Forster | Mar. 28, 1893 |
| 1,213,150             | Bullis  | Jan. 23, 1917 |
| 2,500,052             | Yackel  | Mar. 7, 1950  |
| 2,657,932             | Blaney  | Nov. 3, 1953  |

OTHER REFERENCES

- Journal of The Franklin Institute, November 1951, vol. 252, No. 5, pp. 373 to 381. (Copy in Div. 17.)  
 General Electric Review, July 1952, vol. 55, No. 4, pp. 70 20, 21, 22 and 61. (Copy in Div. 17.)